

July 28, 1964

R. G. STOLL ET AL

3,142,109

FABRICS

Filed Nov. 27, 1959



## 1

3,142,109  
FABRICS

Reiner G. Stoll and Roland A. Frate, Charlotte, N.C.,  
assignors to Celanese Corporation of America, New  
York, N.Y., a corporation of Delaware

Filed Nov. 27, 1959, Ser. No. 855,797  
17 Claims. (Cl. 28—75)

This invention relates to textile fabrics, and in particular to scrim fabrics and to methods of producing the same.

Scrim fabrics are generally characterized by an open or wide mesh structure. It is for this reason that such fabrics very frequently are structurally unstable, i.e., the crossing yarns can shift relative to one another, thereby rendering the mesh arrangement uneven and lessening the utility of such fabrics.

It is an object of the present invention to provide a scrim fabric which is free of these heretofore encountered disadvantages and is both structurally and dimensionally stable and sufficiently strong to withstand stresses in any direction in the plane of the fabric.

Another object of the present invention is the provision of scrim fabrics in which crossing yarn stretches are bonded to one another at the points of intersection thereof without any externally applied adhesive.

Still another object of the present invention is the provision of scrim fabrics as aforesaid in which some of the yarn is composed of a synthetic thermoplastic fiber material capable of being plasticized by a plasticizer, while the remainder of the yarn is composed of a material inert to or not substantially affected by the plasticizer, the adhesion between these yarns at their points of intersection being effected by a rehardening of the thermoplastic yarns after being plasticized and placed in contact with the inert yarns.

A related object of the present invention, therefore, is the provision of such fabrics in which the plasticizer for the thermoplastic yarn is initially carried by the yarn which is inert to the plasticizer.

A further object of the present invention is the provision of a method of producing scrim fabrics as aforesaid which comprises interweaving yarns made of a synthetic thermoplastic fiber material with other yarns which carry a plasticizer for the thermoplastic material.

Yet a further object of the present invention is the provision of a method of producing scrim fabrics which comprises the bonding of yarns to each other at their crossover or intersection points without any external application of an adhesive or bonding material as such. To this end, the fabric is composed partly of yarns of a thermoplastic, plasticizable material and partly of yarns of a different material which is inert to and thus adapted to act as a carrier for a plasticizer for the thermoplastic material. The bond thus is produced by the indirect plasticization of the thermoplastic material and the subsequent hardening thereof. The bond may be completed by a heating operation.

The thermoplastic yarns may be composed in whole or in part of plasticizable fibers, representative examples of which include polyamides such as nylon, polyesters such as polyethylene terephthalate, acrylonitrile polymers and copolymers, and olefin and olefinic ester polymers and copolymers such as polyethylene, polypropylene, polyvinyl

## 2

chloride, polyvinyl acetate, and the like. Especially good results are achieved with organic acid esters of cellulose such as cellulose acetate, cellulose propionate, cellulose butyrate, cellulose acetate formate, cellulose acetate propionate, cellulose acetate butyrate, and the like. Of these, cellulose acetate is preferred.

The other yarns employed in the fabric may comprise fibrous materials similar to those set forth above with the proviso that these materials must be substantially inert to or unaffected by plasticizers for the thermoplastic yarns. In accordance with one aspect of the present invention, these inert yarns may comprise cellulose, e.g. cotton or rayon, preferably high tenacity rayon having a tenacity in excess of about 5.0 grams per denier, such as is obtained by saponification of cellulose acetate. In any given fabric, therefore, the yarns carrying the plasticizer for the thermoplastic yarns will have a different composition than the latter so that the plasticizer will selectively act on only these yarns and cause them to adhere to the inert carrier yarns at the crossover points.

The plasticizer employed in accordance with the present invention may be of any suitable composition and may or may not be volatile. For example, if the thermoplastic fiber yarn is cellulose acetate and the other yarn cellulose, i.e., cotton or high tenacity rayon, the bonding may be best effected by means of plasticizers such as high boiling organic esters of carboxylic acids such as alkyl or aryl esters of citric acid, adipic acid, maleic acid and phthalic acid, organic esters of inorganic acids such as tributyl phosphate and tricresyl phosphate, alkoxy alkyl esters of inorganic polybasic acids or organic polybasic acids, high boiling ethers such as butyl ether of ethylene glycol, methyl ether of ethylene glycol, etc., and high boiling esters of polyhydric alcohols such as triacetin, glycol diacetate and diacetin. The plasticizer may be diluted with water, alcohol or other poor swelling agents to regulate the degree of plasticization of the thermoplastic fiber yarns. Preferably the plasticizer is incorporated in the inert yarns by a coating technique, e.g., by an immersion, dipping or spraying operation, or by being passed over one or more kiss rolls. If necessary, this may be followed by a wiping operation to remove excess liquid so as to prevent dripping. The amount of plasticizer carried by the inert yarns will depend upon the spacing and relative weight of the thermoplastic yarns as well as upon the activity of the particular plasticizer and its concentration. The plasticizer may also comprise a solvent for the thermoplastic material which, under the prevailing circumstances, is incapable of effecting any appreciable dissolution, e.g. it is applied in very small proportion relative to the thermoplastic material or it is employed diluted with non-solvents. In the event such a solvent is employed preferably it is volatile, such as acetone, methylene chloride or the like for cellulose esters, since upon evaporation the bond will be of increased strength.

The thermoplastic and inert yarns may be combined with one another into the desired fabric form by any suitable intermeshing operation such as regular or leno weaving, knitting, e.g., warp knitting, or the like. In accordance with one aspect of the present invention, the inert yarns are taken from a warp beam and passed over a small kiss roll arranged in advance of the drop wires of a loom, whereby the plasticizer is applied to these yarns by surface contact. An electric heating device is ar-

ranged on the loom adjacent the exit path of movement of the fabric so as to heat the intersecting yarns and to complete the bonding initiated by the plasticization of the filling or weft yarns by the plasticizer carried by the warp yarns.

The foregoing and other objects, characteristics and advantages of the present invention will be more fully understood from the following detailed description thereof when read in conjunction with the accompanying drawing, in which:

FIG. 1 is a diagrammatic illustration of an arrangement for forming a bonded scrim fabric according to the present invention; and

FIG. 2 is a diagrammatic plan view of a scrim fabric formed by the device shown in FIG. 1.

Referring first to FIG. 2, it will be seen that the scrim fabric 10 according to the present invention comprises a plurality of warp yarns 11 interwoven with weft or filling yarns 12. The warp yarns 11 are desirably cotton or rayon, preferably high tenacity rayon having a tenacity in excess of about 5.0 grams per denier. The yarns 12, on the other hand, are composed of a synthetic thermoplastic fiber material, cellulose acetate being preferred. The yarns 11 and 12 are bonded to one another at their crossover or intersection points 13 by virtue of the fact that the warp yarns 11 prior to the weaving operation carried a plasticizer for the yarns 12 which, consequently, were plasticized upon coming into contact with the warp yarns 11 so as to adhere to the latter.

As shown in FIG. 1, the warp yarns 11 may be unwound from a warp beam 14 and passed over a small kiss roll 15 partially immersed in a quantity of any suitable plasticizer 16. The portions of the yarns 11 at the location 11a thus are coated or impregnated with the plasticizer 16 which, of course, has no softening effect on the material of which the yarns 11 are made. In this condition, the warp yarns 11 are fed into a loom or similar fabric-forming device 17 in which they are interwoven by conventional means (not shown) with the filling yarns 12. The latter, as hereinbefore stated, become plasticized upon coming into contact with the warp yarns 11 due to the migration of the plasticizer and thus tend to adhere to the warp yarns. After the fabric has been formed, it is subjected to the action of an electric heating device 18 mounted on the loom 17, which effects a completion of the bonds between the yarns 11 and 12. The completed fabric 10 is then removed from the loom and wound up on any suitable take-up roll 19 on which it may be stored and shipped to the ultimate consumer.

It will be understood, of course, that the arrangement may be reversed, with warp yarns being made of thermoplastic fiber materials while the filling yarns are made of materials inert to the plasticizers for the warp yarns. Moreover, the yarns which are to be plasticized need not be made completely of a thermoplastic fiber material, the only requirement being that they contain some plasticizable material. The other yarns, i.e., those carrying the plasticizer, must, however, be composed solely of materials not substantially affected by the plasticizer.

Scrim fabrics produced in accordance with the present invention are suited for use as backings or embedded reinforcements for non-wovens, as sanitary napkin coverings, surgical bandages and other medical uses, and the like.

The invention is further illustrated in the following example.

#### Example

A fabric having 18 ends and 18 picks per inch is woven from 60/2.5/80 high tenacity rayon warp and 100/2/26 cellulose acetate filling. On the way to the loom the warps pick up 50% of their weight of a 30% aqueous solution of diacetin. Following weaving, the scrim fabric is heated over a radiant electric heater to 220° F. and is then taken up on a roll.

It is to be understood that the foregoing detailed description is given merely by way of illustration and that many variations may be made therein without departing from the spirit of our invention.

Having described our invention what we desire to secure by Letters Patent is:

1. A textile fabric, comprising intersecting and intermeshed first and second yarns which are separate along most of their lengths, said first yarns at least partly comprising a thermoplastic fiber material capable of being plasticized by a plasticizer, all the material making up said second yarns being substantially inert to said plasticizer, said first and second yarns being bonded to one another at their crossover points by the action of said plasticizer which is substantially non-adhesive and is initially carried by said second yarns.
2. A textile fabric according to claim 1, wherein said first yarns are composed entirely of said thermoplastic fiber material.
3. A textile fabric according to claim 1, said second yarns comprising rayon having a tenacity of at least 5.0 grams per denier.
4. A textile fabric according to claim 1, said thermoplastic fiber material comprising cellulose acetate.
5. A textile fabric according to claim 1, said thermoplastic fiber material comprising nylon.
6. A scrim fabric, comprising intersecting and intermeshed thermoplastic fiber yarns and other yarns which are separate along most of their lengths and are bonded to one another at their crossover points by the action of a plasticizer for said thermoplastic fiber yarns which is substantially non-adhesive and is initially carried by said other yarns, all the material making up said other yarns being substantially inert to said plasticizer.
7. A scrim fabric according to claim 6, said thermoplastic fiber yarns and said other yarns intermeshing with one another by weaving.
8. A scrim fabric according to claim 6, said thermoplastic fiber yarns and said other yarns intermeshing with one another by knitting.
9. A scrim fabric according to claim 6, wherein said thermoplastic fiber yarns comprise an organic acid ester of cellulose.
10. A scrim fabric according to claim 6, wherein said thermoplastic fiber yarns comprise cellulose acetate.
11. A scrim fabric according to claim 6, wherein said other yarns comprise cellulose.
12. A scrim fabric according to claim 11, wherein said other yarns comprise rayon having a tenacity of at least 5.0 grams per denier.
13. The method of forming a textile fabric, comprising the steps of intermeshing first yarns at least in part comprising a thermoplastic fiber material capable of being plasticized by a plasticizer with second yarns, all the material making up said second yarns being substantially inert to said plasticizer, and applying said plasticizer to said second yarns prior to the intermeshing thereof with said first yarns, whereby following intermeshing said first and second yarns are bonded to one another at their crossover points by the action of said plasticizer on said first yarns.
14. The method of claim 13, further including the step of heating said first and second yarns subsequent to the intermeshing thereof for improving the bond therebetween.
15. The method of claim 13, wherein said intermeshing step comprises weaving said first and second yarns on a loom.
16. The method of claim 13, wherein said intermeshing step comprises knitting said first and second yarns on a knitting machine.
17. The method of claim 13, wherein the thermoplastic fiber material of which said first yarns are made comprises cellulose acetate.

## References Cited in the file of this patent

| UNITED STATES PATENTS |                                 |
|-----------------------|---------------------------------|
| 1,421,498             | Koch ----- July 4, 1922         |
| 2,081,620             | Fether ----- May 25, 1937       |
| 2,308,593             | Brew ----- Jan. 19, 1943        |
| 2,342,231             | Whitehead ----- Feb. 22, 1944   |
| 2,460,674             | Bihaly ----- Feb. 1, 1949       |
| 2,536,163             | Feild et al. ----- Jan. 2, 1951 |
| 2,864,151             | Bihaly ----- Dec. 16, 1953      |

|           |
|-----------|
| 2,757,435 |
| 2,771,659 |
| 2,811,029 |
| 2,900,980 |

|                             |
|-----------------------------|
| Bihaly ----- Aug. 7, 1956   |
| Ball ----- Nov. 27, 1956    |
| Conner ----- Oct. 29, 1957  |
| Harwood ----- Aug. 25, 1959 |

## FOREIGN PATENTS

|                                   |
|-----------------------------------|
| Canada ----- Dec. 30, 1958        |
| Great Britain ----- Sept. 7, 1943 |
| Great Britain ----- Mar. 4, 1959  |